

1

3,692,663

## PROCESS FOR TREATING TARS

Koza Ueda, Kyoto, Jitsumi Kimoto, Takarazuka, and  
Mitsuru Moritake, Saita, Japan, assignors to Osaka  
Gas Company, Limited, Osaka-shi, Japan

No Drawing. Filed Mar. 19, 1971, Ser. No. 126,356

Int. Cl. C10c 3/02

U.S. Cl. 208—44

8 Claims

### ABSTRACT OF THE DISCLOSURE

The process for treating tars of this invention comprises steps of (1) heating a starting tar to a temperature of 320 to 470° C. under increased pressure of 1 to 20 kg./cm.<sup>2</sup> gauge to produce gas, oil and pitch, (2) separating oil and pitch by distillation to produce pitch having a softening point of at least 60° C. and containing 20 to 45% by weight of benzene-insoluble content and 3 to 20% by weight of quinoline-insoluble content, (3) heating the resulting oil under increased pressure of 3 to 35 kg./cm.<sup>2</sup> gauge at a temperature ranging from 370 to 540° C. and at least 10° C. higher than the heating temperature in the first step to produce gas, oil and pitch, and (4) separating oil and pitch by distillation to produce pitch having a softening point of at least 60° C. and containing 15 to 40% by weight of benzene-insoluble content and not more than 2% by weight of quinoline-insoluble content.

This invention relates to a novel process for treating tars.

In general, tar resulting from dry distillation of coal or cracking of petroleum is treated principally for the purpose of recovering oils, and pitch is obtained as a resulting byproduct. In most tar industries, tar is subjected to distillation under atmospheric or reduced pressure to obtain light, middle and heavy fractions for use as industrial materials and a residue is recovered as pitch. The resulting pitch is utilized as a binder for producing electrodes, as an impregnating agent for baked electrodes to improve mechanical and electric properties of the electrodes and as an additive to be added to coking coal charge in producing coke to improve the qualities of the coke. However, the pitch produced by such method has limited properties with the result that the pitch can be used only for the restricted applications and purposes.

The properties of pitch are generally represented by solubility in solvents: pitch is divided into benzene-soluble content and benzene-insoluble content, the benzene-insoluble content further being divided into quinoline-soluble and quinoline-insoluble contents. Pitch obtained by conventional methods generally has a softening point in excess of 60° C. and contains 20 to 40% by weight of benzene-insoluble content and 5 to 20% by weight of quinoline-insoluble content. With respect to such properties, increase in benzene-insoluble content inevitably results in greater quinoline-insoluble content. On the contrary, if it is attempted to lower the quinoline-insoluble content, the benzene-insoluble content will also be lowered with increased benzene-soluble content. In many cases, however, the amount of both benzene-insoluble content and quinoline-insoluble content, and the difference between these two amounts are critical factors to determine the properties of pitch. For instance, if it is desired to obtain an electrode having improved properties in strength, density and specific electric resistance by using pitch as a binding agent, it is required that the pitch have at least 30% by weight of benzene-insoluble content and low quinoline-insoluble content and that the component (so-called  $\beta$ -resin) accounting for the difference between the benzene-

2

insoluble content and the quinoline-insoluble content be at least 20% by weight. Notwithstanding this, it has been difficult to obtain pitch satisfying such requirements, since an attempt to increase benzene-insoluble content to more than 30% by weight is accompanied by a corresponding increase in quinoline-insoluble content. Further it is desired that pitch to be used as an impregnating agent for baked electrodes have the lowest possible quinoline-insoluble content. More specifically, it is required for the pitch to contain not more than 3% by weight of quinoline-insoluble content and at least 20% by weight of benzene-insoluble content. With a conventional method, however, preparation of pitch having not more than 3% by weight of quinoline-insoluble content encounters a consequent difficulty that the benzene-insoluble content lowers to about 15% by weight or less with a predominant amount being benzene-soluble content, this making it impossible to obtain pitch for use as an impregnating agent which has desired properties. Thus, with conventional method, pitch obtained had restricted properties and it was impossible to control properties of pitch as desired in conformity with various uses and purposes.

An object of this invention is to provide a process by which pitch useful for a wide variety of applications can be recovered in high yield by treating tars under increased pressure unlike conventional distillation treatment and by which thermally stable oils having excellent qualities and gases employable as a fuel source can also be recovered.

Another object of this invention is to provide a process for treating tars by which amounts of benzene-insoluble content and quinoline-insoluble content can be controlled individually and which is therefore capable of providing pitch satisfying every requirement involved in various uses and purposes.

Another object of this invention is to provide a process for treating tars whereby useful pitch having peculiar characteristics can be prepared by each step of multi-step heat treatment and by mixing respective pitches obtained by respective steps.

Another object of this invention is to provide a process for treating tars whereby pitch can be obtained in high yield of at least 75% by weight based on tars without coking difficulties.

Still another object of this invention is to provide a process for treating tars which is capable of producing oil of high quality almost free of unstable components as byproduct.

The above and other objects of this invention will become more apparent from the following description.

The process for treating tars of this invention comprises steps of (1) heating a starting tar to a temperature of 320 to 470° C. under increased pressure of 1 to 20 kg./cm.<sup>2</sup> gauge to produce gas, oil and pitch, (2) separating oil and pitch by distillation to produce pitch having a softening point of at least 60° C. and containing 20 to 45% by weight of benzene-insoluble content and 3 to 20% by weight of quinoline-insoluble content, (3) heating the resulting oil under increased pressure of 3 to 35 kg./cm.<sup>2</sup> gauge at a temperature ranging from 370 to 540° C. and at least 10° C. higher than the heating temperature in the first step to produce gas, oil and pitch, and (4) separating oil and pitch by distillation to produce pitch having a softening point of at least 60° C. and containing 15 to 40% by weight of a benzene-insoluble content and not more than 2% by weight of quinoline-insoluble content.

The softening point as used in this specification and claims is a value determined in accordance with mercury method set forth in JIS (Japanese Industrial Standards) K 2421-66.

In accordance with this invention, tar is heated under increased pressure during two steps of heat treatment, whereby pitch having particular characteristics can be obtained by each step of heat treatment operation. More specifically, when tar is heated to 320 to 470° C. directly under increased pressure of 1 to 20 kg./cm.<sup>2</sup> gauge, pitch containing 20 to 45% by weight of benzene-insoluble content and 3 to 20% by weight of quinoline-insoluble content can be obtained in high yield together with gas and oil. Pitch having such properties fully meets the requirements of various uses and can be used as a binder for electrodes, an impregnating agent for baked electrodes and an additive for coal. Although increase of the benzene-insoluble content may result in increase of quinoline-insoluble content, the increase is much smaller than is the case with the conventional method. Even where the benzene-insoluble content exceeds 30% by weight, at least 23% by weight of the  $\beta$ -resin component can be retained, this showing a particular advantage that the pitch can be used as a binder in producing electrodes having more excellent properties than conventionally possible. In fact, in the case where pitch prepared in accordance with this invention and containing  $\beta$ -resin content exceeding 23% by weight is used as a binder, electrodes produced have improved bending strength, compression strength and specific electric resistance. The fact that pitch with such properties can be obtained is attributable solely to the foregoing heat treatment which is carried out under increased pressure so as to positively convert effective components in tar to pitch. Such result can not be obtained by conventional methods of distillation wherein treatment is conducted under atmospheric or reduced pressure.

In accordance with the present invention, oil resulting from the first step of heat treatment is then treated under severer conditions than in the first step, whereby pitch containing a very low quinoline-insoluble content is prepared. Despite the fact that pitch obtained by the second step of heat treatment contains 15 to 40% by weight of benzene-insoluble content, the amount of quinoline-insoluble content is even lower than 2% by weight. Such pitch is very suitable for uses wherein a sufficiently great amount of benzene-insoluble content and a relatively small amount of quinoline-insoluble content are essential as in the case of impregnating agent for baked electrodes. A baked electrode impregnated with pitch of this invention having a low quinoline-insoluble content has exceedingly improved bending strength, compression strength and specific electric resistance. Moreover, since the pitch resulting from the first step of heat treatment is distinct from the pitch obtained from the second step of heat treatment in properties, especially in quinoline-insoluble content, both pitches, when mixed together, can be formed into pitch of desired properties. Thus, the pitch of this invention can be applied to wider uses and purposes because of excellent properties. In addition, since the oil from the first step of heat treatment is converted into pitch in the second step of heat treatment, the total yield of pitch can be substantially increased and the oil product obtained only from the second step of heat treatment is almost free of unstable components. A high quality oil very useful as an absorbent will be thus produced. In accordance with this invention wherein tar is converted to pitch by a two-step heat treatment, it is possible to convert unstable components to pitch through the first step of heat treatment so that coking will not be likely to take place nor will troubles arise in operation or in apparatus even when the products are treated under severer conditions during the second step of heat treatment.

The softening point of pitch obtained from each step of heat treatment can be adjusted over a wide range as desired by varying heat treatment conditions as well as conditions of distillation conducted after the heat treatment, namely by varying the amount of low-boiling frac-

tion. Generally, the softening point of pitch is in the range of about 60 to 150° C., though it is possible to obtain pitch having higher softening point of 150 to 300° C.

The tars to be used as starting material of this invention include coal-tar and oil gas tar produced by thermal or catalytic cracking of petroleum, the tars being such that they have an absolute viscosity of 20 to 1000 centipoises at 50° C. and containing 5 to 30% by weight of 0-270° C. fraction and 25 to 45% by weight of 0-360° C. fraction. Particularly preferable are tars having an absolute viscosity of 50 to 200 centipoises at 50° C. and containing 15 to 25% by weight of 0-270° C. fraction and 30 to 40% by weight of 0 to 360° C. fraction.

In accordance with the method of the present invention the starting tar is heated to 320 to 470° C. under increased pressure of 1 to 20 kg./cm.<sup>2</sup> gauge, whereby effective components in the starting tar are positively converted to pitch. More specifically, heavy fraction and relatively low-boiling, unstable condensed ring substances undergo condensation polymerization to be converted to pitch, while unreacted components are obtained as an oil fraction together with a gaseous reaction product. During this step, the reaction temperature of 320 to 470° C. is of important significance: a temperature lower than 320° C. fails to effect the reaction satisfactorily, whereas a temperature in excess of 470° C. gives rise to coking in the reactor. The reaction may preferably be carried out at a temperature of 380 to 430° C. It is required to effect the reaction in this step under increased pressure of 1 to 20 kg./cm.<sup>2</sup> gauge, whereby the substances to be reacted in the tar can be retained in a liquid phase to insure positive conversion to pitch. There is a need to avoid treatment under an atmospheric or reduced pressure, because such treatment would allow relatively low-boiling, unstable condensed ring substances to be left unreacted without subjecting the substances to condensation polymerization for conversion to pitch, this not only preventing formation of pitch with good quality but causing coking within the reactor during the second step of heat treatment conducted under severe reaction conditions. On the contrary, when the pressure exceeds 20 kg./cm.<sup>2</sup> gauge, better results will not be achieved and troubles will be encountered with apparatus and operation. Suitable pressure for the reaction at this stage is therefore in the range of 5 to 15 kg./cm.<sup>2</sup> gauge. The reaction time may vary over a wide range depending upon the reaction conditions and properties of pitch to be obtained, but usually the reaction is completed in about 1 to 20 hours.

The first step of heat treatment results in the production of gas, oil and pitch. The gas is taken out from the system for the use in fuel source and the resulting mixture of oil and pitch is subjected to distillation for separation. The pitch thus obtained has a softening point of at least 60° C. and containing 20 to 45% by weight of benzene-insoluble content and 3 to 20% by weight of quinoline-insoluble content.

Oil obtained in the first step of heat treatment is further heated in the subsequent second step of heat treatment, wherein reaction is effected at a temperature at least 10° C. higher than that applied in the first step of heat treatment. During this step, components left unreacted in the preceding heat treatment step are positively converted to pitch. The reaction temperature is in the range of 370 to 540° C., while the reaction pressure is 3 to 35 kg./cm.<sup>2</sup> gauge. Reaction temperature lower than that in the first step of heat treatment or below 370° C. retards reaction for conversion to pitch, making it difficult to obtain desired pitch, whereas a temperature exceeding 540° C. gives rise to coking. The reaction temperature may preferably be in the range of 420 to 460° C., which is 30 to 60° C. higher than that applied in the first heat treatment step. Further reaction pressure lower than 3 kg./cm.<sup>2</sup> gauge will cause low-boiling components to evaporate off and deteriorate pitch yield, producing adverse effects on properties. On the other hand, a pressure exceeding 35

kg./cm.<sup>2</sup> gauge will merely cause troubles to apparatus or result in difficulties in operation without producing any improvement in efficiency. The pressure may preferably be

7 to 20 kg./cm.<sup>2</sup> gauge. The reaction for the second heat treatment step is generally completed in 1 to 40 hours although the reaction time varies over a wide range depending upon the reaction conditions and the properties of pitch to be produced.

In the second heat treatment step gas, oil and pitch are obtained, and during the operation gas is taken out from the system for the use in fuel source. The resulting mixture of oil and pitch is subjected to distillation for separation. The pitch obtained from this step has a softening point of at least 60° C. and peculiar properties in that it contains 15 to 40% by weight of benzene-insoluble content and an exceedingly small amount of, i.e. not more than 2% by weight of, quinoline-insoluble content. It has been impossible for a conventional method to produce such pitch that contains very small amount of quinoline-insoluble content in spite of high-benzene-insoluble content which amounts to 15 to 40% by weight. Indeed, the pitch thus prepared finds versatile applications, for instance, as an impregnating agent for baked electrodes. This invention further has a particular advantage that the pitch obtained by the second heat treatment step can be mixed with the pitch prepared by the first heat treatment step to readily prepare pitch of desired properties. The oil obtained by the present process has excellent thermal stability and is used as good absorbent since unstable components have been converted to pitch by the two steps of heat treatment.

The present invention has been described with respect to a case wherein tar is treated by two steps of heat treatment operation. However, in accordance with this invention tar can further be treated by a multi-step heat treatment. That is, the oil produced by the second heat treatment step will then be treated thermally under severer conditions, for instance, at a temperature ranging from 380 to 560° C. and at least 10° C. higher than that in the second step under a pressure of 3 to 35 kg./cm.<sup>2</sup> gauge. Pitch produced by such multi-step heat treatment has peculiar properties and contains much lower quinoline-insoluble content. It is desired to employ such multi-step heat treatment depending upon requirements in uses of pitch.

The method of the invention can be conducted by batch method as well as in continuous manner.

For a better understanding of the invention examples are given below, in which percentages are by weight.

#### EXAMPLE 1

Crude coal tar was passed through a wetted-wall tower at 84° C. to remove water contained therein. The dried tar had an absolute viscosity at 50° C. of 102.4 cps. and contained 17.1% of a fraction boiling at 0 to 270° C. and 36.8% of a fraction boiling at 0 to 360° C. The tar was placed in an autoclave equipped with a partial condenser and pressure regulator and heated at 400° C. under 9 kg./cm.<sup>2</sup> gauge for 5 hours. The vapor produced was condensed in the partial condenser for refluxing and non-condensed gas was taken out from the system. The tar thus treated was subjected to isothermal flash distillation to separate pitch and oil.

The yields of the pitch, oil and gas thus obtained and the properties of the pitch are shown in Table 1.

The oil obtained in the first heat treatment step was then placed in an autoclave with a partial condenser and pressure regulator. The oil in the autoclave was heated at 450° C. under 12 kg./cm.<sup>2</sup> gauge for 10 hours. The vapor produced was condensed in the partial condenser for refluxing and non-condensed gas was taken out of the system. Oil thus treated was subjected to isothermal flash distillation to separate pitch and oil.

The yields of the pitch, oil and gas thus obtained and the properties of the pitch and oil are shown in Table 1 below.

TABLE 1

|    |                                              | First<br>heat<br>treat-<br>ment<br>step | Second<br>heat<br>treat-<br>ment<br>step |
|----|----------------------------------------------|-----------------------------------------|------------------------------------------|
| 10 | Yield (percent):                             |                                         |                                          |
|    | Pitch.....                                   | 64.0                                    | 45.5                                     |
|    | Oil.....                                     | 35.1                                    | 52.4                                     |
|    | Gas.....                                     | 0.9                                     | 2.1                                      |
| 15 | Properties: pitch:                           |                                         |                                          |
|    | Softening point (° C.).....                  | 80.5                                    | 81.0                                     |
|    | Volatile substance (percent).....            | 45.8                                    | 46.9                                     |
|    | Quinoline-insoluble content (percent).....   | 7.2                                     | 0.7                                      |
|    | Benzene-insoluble content (percent).....     | 32.0                                    | 28.7                                     |
| 20 | Properties: oil:                             |                                         |                                          |
|    | Specific gravity.....                        | 1.05                                    |                                          |
|    | Temperature for 20% distillation (° C.)..... | 221                                     |                                          |
|    | Temperature for 50% distillation (° C.)..... | 252                                     |                                          |
|    | Temperature for 80% distillation (° C.)..... | 336                                     |                                          |
|    | Acenaphthene content (percent).....          | Trace                                   |                                          |

#### EXAMPLE 2

Dried coal tar the same as in Example 1 was heat-treated under the same conditions as in Example 1, and the oil obtained in the second heat treatment step was then placed in an autoclave equipped with a partial condenser and pressure regulator and heated at 460° C. under a pressure of 20 kg./cm.<sup>2</sup> gauge for 20 hours. The product thus treated was subjected to flash distillation to separate pitch and oil. The yield of the pitch based on the weight of the oil from the second step was 36.5%, and the properties thereof are shown in Table 2 below.

TABLE 2

|    |                                             |      |
|----|---------------------------------------------|------|
| 35 | Softening point (° C.) .....                | 82   |
|    | Quinoline-insoluble content (percent) ..... | 0.2  |
|    | Benzene-insoluble content (percent) .....   | 15.2 |

#### EXAMPLE 3

40 Dried coal tar the same as in Example 1 was heat-treated in the same manner as in Example 1, except that the conditions applied in the first and second heat treatment steps were changed as shown in Table 3 below, in which are also disclosed the properties of the pitch and oil obtained in respective steps.

TABLE 3

|    |                                              | First<br>heat<br>treat-<br>ment<br>step | Second<br>heat<br>treat-<br>ment<br>step |
|----|----------------------------------------------|-----------------------------------------|------------------------------------------|
| 50 | Conditions:                                  |                                         |                                          |
|    | Temperature (° C.).....                      | 360                                     | 430                                      |
|    | Pressure (kg./cm. <sup>2</sup> G).....       | 5                                       | 8                                        |
|    | Time (hours).....                            | 18                                      | 20                                       |
| 55 | Yield, percent:                              |                                         |                                          |
|    | Pitch.....                                   | 55.1                                    | 61.1                                     |
|    | Oil.....                                     | 44.6                                    | 37.2                                     |
|    | Gas.....                                     | 0.3                                     | 1.7                                      |
| 60 | Properties: pitch:                           |                                         |                                          |
|    | Softening point (° C.).....                  | 76.0                                    | 70.5                                     |
|    | Volatile substance (percent).....            | 48.2                                    | 47.3                                     |
|    | Quinoline-insoluble content (percent).....   | 8.4                                     | 1.6                                      |
|    | Benzene-insoluble content (percent).....     | 35.2                                    | 28.1                                     |
| 65 | Properties: oil:                             |                                         |                                          |
|    | Specific gravity.....                        | 1.04                                    |                                          |
|    | Temperature for 20% distillation (° C.)..... | 217                                     |                                          |
|    | Temperature for 50% distillation (° C.)..... | 248                                     |                                          |
|    | Temperature for 80% distillation (° C.)..... | 330                                     |                                          |
|    | Acenaphthene content (percent).....          | Trace                                   |                                          |

#### EXAMPLE 4

70 Dried coal tar the same as in Example 1 was heat-treated in the same manner as in Example 1, except that the conditions applied in the first and second treatment steps were changed as shown in Table 4 below, in which are also disclosed the properties of the pitch and oil obtained in respective steps.

7  
TABLE 4

|                                         | First<br>heat<br>treat-<br>ment<br>step | Second<br>heat<br>treat-<br>ment<br>step |    |
|-----------------------------------------|-----------------------------------------|------------------------------------------|----|
| Conditions:                             |                                         |                                          |    |
| Temperature (° C.)                      | 460                                     | 490                                      |    |
| Pressure (kg./cm. <sup>2</sup> G.)      | 20                                      | 20                                       |    |
| Time (hours)                            | 2                                       | 2                                        |    |
| Yield:                                  |                                         |                                          | 5  |
| Pitch                                   | 71.2                                    | 40.6                                     |    |
| Oil                                     | 26.0                                    | 57.0                                     | 10 |
| Gas                                     | 2.8                                     | 2.4                                      |    |
| Properties; pitch:                      |                                         |                                          |    |
| Softening point (° C.)                  | 85.3                                    | 84.5                                     |    |
| Volatile substance (percent)            | 44.3                                    | 49.0                                     |    |
| Quinoline-insoluble content (percent)   | 10.5                                    | 0.1                                      |    |
| Benzene-insoluble content (percent)     | 36.1                                    | 20.3                                     |    |
| Properties; oil:                        |                                         |                                          | 15 |
| Specific gravity                        |                                         | 1.08                                     |    |
| Temperature for 20%-distillation (° C.) |                                         | 231                                      |    |
| Temperature for 50%-distillation (° C.) |                                         | 250                                      |    |
| Temperature for 80%-distillation (° C.) |                                         | 334                                      |    |
| Acenaphthene content (percent)          |                                         | Trace                                    |    |

## EXAMPLE 5

Crude oil gas tar was dried in the same manner as in Example 1 to obtain dried tar having an absolute viscosity at 50° C. of 28.7 cps. and containing 20.3% of a fraction boiling at 0 to 270° C. and 35.0% of a fraction boiling at 0 to 360° C. The dried tar was then subjected to the heat treatment in the same manner as in Example 1, except that the conditions applied in the first and second heat treatment steps were changed as shown in Table 5 below, in which are also shown the properties of the pitch and oil obtained in each step.

TABLE 5

|                                         | First<br>heat<br>treat-<br>ment<br>step | Second<br>heat<br>treat-<br>ment<br>step |    |
|-----------------------------------------|-----------------------------------------|------------------------------------------|----|
| Conditions:                             |                                         |                                          | 40 |
| Temperature (° C.)                      | 385                                     | 450                                      |    |
| Pressure (kg./cm. <sup>2</sup> G.)      | 9                                       | 9                                        |    |
| Time (hours)                            | 5                                       | 10                                       |    |
| Yield; (percent):                       |                                         |                                          | 45 |
| Pitch                                   | 59.3                                    | 48.6                                     |    |
| Oil                                     | 39.6                                    | 48.0                                     |    |
| Gas                                     | 0.7                                     | 3.4                                      |    |
| Properties; pitch:                      |                                         |                                          | 50 |
| Softening point (° C.)                  | 79.8                                    | 76.0                                     |    |
| Volatile substance (percent)            | 47.2                                    | 48.0                                     |    |
| Quinoline-insoluble content (percent)   | 8.4                                     | 2.0                                      |    |
| Benzene-insoluble content (percent)     | 34.2                                    | 31.3                                     |    |
| Properties; oil:                        |                                         |                                          | 55 |
| Specific gravity                        |                                         | 1.04                                     |    |
| Temperature for 20%-distillation (° C.) |                                         | 216                                      |    |
| Temperature for 50%-distillation (° C.) |                                         | 247                                      |    |
| Temperature for 80%-distillation (° C.) |                                         | 340                                      |    |
| Acenaphthene content (percent)          |                                         | Trace                                    |    |

For comparison tar was treated in the following manners:

## Comparison I

Coal tar the same as in Example 1 was distilled at 310° C. under atmospheric pressure and the residue was further distilled at 345° C. under reduced pressure of -0.85 kg./cm.<sup>2</sup> gauge. Thus pitch and oil were obtained in yields of 54.9% and 45.1% respectively, based on the weight of the starting coal tar used. The properties thereof are shown in Table 6 below.

TABLE 6

|                                         |       |  |    |
|-----------------------------------------|-------|--|----|
| Pitch                                   |       |  |    |
| Softening point (° C.)                  | 67.7  |  |    |
| Volatile substance (percent)            | 50.7  |  |    |
| Quinoline-insoluble substance (percent) | 4.1   |  |    |
| Benzene-insoluble substance (percent)   | 18.2  |  |    |
| Oil:                                    |       |  | 70 |
| Specific gravity                        | 1.08  |  |    |
| Temperature for 20%-distillation (° C.) | 240.5 |  |    |
| Temperature for 50%-distillation (° C.) | 325   |  |    |
| Temperature for 80%-distillation (° C.) | 360   |  |    |
| Acenaphthene content (percent)          | 0.80  |  |    |

75

8  
Comparison II

The pitch obtained in Comparison I was further heated at 400° C. under atmospheric pressure for 5 hours. The properties of the pitch thus obtained are shown in Table 7 below.

## Table 7

|                                     |      |
|-------------------------------------|------|
| Softening point (° c.)              | 82   |
| Quinoline-insoluble content percent | 17.1 |
| Benzene-insoluble content percent   | 37.0 |

## Comparison III

The oil obtained from distillation under reduced pressure in Comparison I and having the following properties was subjected to heat treatment under the same conditions as applied in the second step of heat treatment in Example 1. During the treatment coking occurred to produce rigid solid containing 82.0% of quinoline-insoluble content in a yield of 13% based on the weight of the oil used.

The properties of the oil used were as follows:

|                                  |                |     |
|----------------------------------|----------------|-----|
| Absolute viscosity               | cps. at 80° C. | 5.8 |
| Content of 0 to 270° C. fraction | percent        | 0   |
| Content of 0 to 360° C. fraction | percent        | 50  |

What we claim is:

1. A process for treating tar which comprises steps of:
  - (1) heating starting tar to a temperature of 320 to 470° C. under increased pressure of 1 to 20 kg./cm.<sup>2</sup> gauge to produce gas, oil and pitch,
  - (2) separating oil and pitch by distillation to obtain pitch having a softening point of at least 60° C. and containing 20 to 45% by weight of benzene-insoluble content and 3 to 20% by weight of quinoline-insoluble content,
  - (3) heating the resulting oil under increased pressure of 3 to 35 kg./cm.<sup>2</sup> gauge at a temperature ranging from 370 to 540° C. and at least 10° C. higher than the heating temperature in the first step to produce gas, oil and pitch, and
  - (4) separating oil and pitch by distillation to obtain pitch having a softening point of at least 60° C. and containing 15 to 40% by weight of benzene-insoluble content and not more than 2% by weight of quinoline-insoluble content.
2. The process according to claim 1, in which said tar has an absolute viscosity at 50° C. of 20 to 1000 cps. and contains 5 to 30% by weight of 0 to 270° C. fraction and 25 to 45% by weight of 0 to 360° C. fraction.
3. The process according to claim 2, in which said tar has an absolute viscosity at 50° C. of 50 to 200 cps. and contains 15 to 25% by weight of 0 to 270° C. fraction and 30 to 40% by weight of 0 to 360° C. fraction.
4. The process according to claim 1, in which said first heat treatment step for the starting tar is conducted at a temperature of 380 to 430° C. under increased pressure of 5 to 15 kg./cm.<sup>2</sup> gauge.
5. The process according to claim 1, in which said second heat treatment step for the oil resulting from said first heat treatment step is conducted at a temperature of 420 to 460° C. under increased pressure of 7 to 20 kg./cm.<sup>2</sup> gauge.
6. The process according to claim 5, in which said temperature in the second heat treatment step is a temperature of 30 to 60° C. higher than that applied in the first heat treatment step.
7. The process according to claim 1, in which said pitch obtained in the first heat treatment step is mixed with the pitch obtained in the second heat treatment step to adjust the properties of the pitch.
8. The process according to claim 1, in which said oil obtained from the second heat treatment step is further heat-treated under increased pressure of 3 to 35 kg./cm.<sup>2</sup> gauge at a temperature ranging from 380 to 560° C. and

3,692,663

9

at least 10° C. higher than the heating temperature in the second-step heat treatment.

10

FOREIGN PATENTS

628,474 10/1961 Canada ----- 208—44

References Cited

UNITED STATES PATENTS

|           |        |                     |          |        |
|-----------|--------|---------------------|----------|--------|
| 2,985,577 | 5/1961 | Geller et al. ----- | 208—44 X | 5      |
| 2,992,181 | 7/1961 | Renner -----        | 208—44 X | 208—22 |
| 3,190,812 | 6/1965 | Puls -----          | 208—44 X |        |

DELBERT E. GANTZ, Primary Examiner

U.S. CL. X.R.

UNITED STATES PATENT OFFICE  
CERTIFICATE OF CORRECTION

Patent No. 3,692,663 Dated September 19, 1972

Inventor(s) Kozo Ueda, Jitsumi Kimoto and Mitsuru Moritake

It is certified that error appears in the above-identified patent and that said Letters Patent are hereby corrected as shown below:

In the heading insert --

Claims priority of Japanese Application Serial No.  
37646/70, filed May 1, 1970.

Signed and sealed this 8th day of May 1973.

(S. M. J.)  
Attest:

ROBERT GOTTSCHALK, JR.  
Attesting Officer

ROBERT GOTTSCHALK  
Commissioner of Patents